

July 1, 1930.

A. C. FISCHER

1,769,635

CONSTRUCTIONAL MATERIAL AND METHOD OF MAKING SAME

Original Filed July 28, 1922



Inventor:  
Albert C. Fischer,  
By Ballard Moore, attorney.

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL AND METHOD OF MAKING SAME

Original application filed July 28, 1922, Serial No. 578,177. Divided and this application filed August 15, 1927. Serial No. 218,193.

My invention relates to a novel and improved constructional material and method of making same, and particularly pertains to a structure having a body of elastic and compressible material reenforced with a surfacing means.

The invention is typified by an expansion joint strip which is constructed for application between rigid elements in building and paving constructions to allow for expansion and contraction.

Heretofore in the art of preparing expansion joints reinforcement has been placed upon the asphaltic body or strip either on one side or both sides of the asphaltic strip, or in the center.

One of the objects of my invention is to provide an improved article and an improved method wherein the reinforcement for the waterproofing material is imbedded or formed in the superficial portion of the walls of the material during the formation of the strip.

Another object of my invention resides in applying fibrous material, preferably relatively long fibers to the sides of the pre-formed strip of waterproofing material, which sides are made adherent so as to hold the fibers in position thereon.

My invention also comprises the step of pressing or imbedding these adherent fibers into the material forming the superficial faces of the strip, whereby to provide an adequate reinforcing means for the strip to hold it in shape and for other purposes hereinafter mentioned.

Another object of my invention resides in providing the strip itself and particularly for forming constructional material of various shapes and sizes.

My invention herein is particularly adapted to the formation of expansion joints and rail filler.

My invention relates particularly to coating the sides of the strip after being pressed into sheet form with varnish or other waterproofed adhesive binder, and by directing against said adhesive binder while in an adhesive state fibrous material which will adhere to said adhesive binder, but which bind-

er will set to a waterproof film, having either imbedded or on the surface of said film the fibrous material or fibers which have been directed against the sides of said joint.

The preferred method of preparing such a strip comprises extruding the bituminous waterproof mass or the waterproofed mixture which is to constitute the body of the strip, and while the strip is thus in a clean state applying or directing vegetable, animal or mineral fibers to the sides of the strip, then pressing said strip between rolls and pressing the fibers so directed against this side into the surface of the strip.

When an asphaltic mass is extruded in an extrusion machine its surface is clean and the mastic exposed, and said fibers may be readily directed against the surfaces thus exposed and pressed into the surfaces, thus giving reinforcing value to the sides of the strip. Or, alternatively, the strip thus extruded or pressed between suitable rolls for the purpose, may be varnished with any suitable varnish, preferably one that dries to a flexible waterproof film, or other waterproofing means may be employed. As an example of the latter I coat a thin film of waterproof adhesive material over the sides of the strip, and the fibers are then directed against and pressed into the surfaces.

I prefer to use asbestos fiber because it is a mineral material and will remain free from decay. However, any suitable fiber having length as distinguished from granular material is suitable; the purpose being to apply the fiber either by shaking it through a screen so that it is applied on the surface, or the fiber, if light enough may be directed by a blast of air against the sides of the strip. It is immaterial how the fiber is applied to the surfaces of the strip provided it is distributed uniformly and in sufficient quantity to add reinforcing value to the side of the strip.

It may be necessary to press the strip after the fiber is directed to the surface. A better surface will be created if the fiber is pressed into the adhesive waterproof film.

This application is a division of my application Serial No. 578,177, filed July 28, 1922, 100

and refers to that part of the application in which asbestos fiber is dusted into adhesive surfaces for the purpose of acting as a reinforcing means and at the same time preventing adhesion of the sides of the joint when packed in a crate.

The body of the expansion joint may be formed by using any waterproofed binder and uniting therewith fillers of various kinds. For instance, it may be a body composed of materials as disclosed in my Reissue Patent No. 16,554, and my Patent No. 1,591,968, patented July 13, 1926, and may be either a homogeneous mixture of fibers between waterproofed binder, or may consist of a homogeneous mixture of flake material and waterproofed binder, or a combination of fiber and flake material, or in fact it may be a plain bituminous mass or a plain waterproofed binder having sufficient body which when reinforced as outlined in this invention, can be handled and will function in a satisfactory manner as an expansion joint. Or the waterproof binder may contain any granular material or mineral filler. I do not wish to be limited to any specific composition of which the main body of the expansion joint is made.

When saturated felt sides have been utilized for expansion joint the fibers are more or less broken down and have not the binding value which the fibers have according to my process and method of preparing the sides of the joint. It can readily be understood that when a very strong and tough setting adhesive is used a very strong reinforcement can be produced. These adhered and pressed in fibers act as a much better reinforcement than saturated felt does during warm weather, and the fact that the fibers are longer and stronger greatly intensifies the strength of the sides. This is especially true of a varnish or a waterproof binder, which does not soften in the warmer temperatures.

In the drawings, Figure 1 illustrates one manner of forming my improved expansion joint, wherein the waterproofed material is rolled into sheet form and has the fibers applied thereto on its upper and lower side.

Figure 2 is a similar diagrammatic view showing the manner of preliminarily coating the sheet of waterproofing material with an adhesive film prior to applying the fibers, preferably by means of an air blast.

Figure 3 is a view of an end of an extruding machine, which constitutes an alternative means for forming the waterproofed material into sheet form.

Figure 4 is a view of a portion of a strip of the finished article formed by adhering the fibers to the tacky surface of the waterproofing material before being set.

Figure 5 is a similar view showing how the fibers are adhered to an adhesive film with

which the waterproofing material is coated; and

Figure 6 is still another view showing the manner of adhering the fibers to an adhesive film with which the waterproofing is coated, the fibers being then coated with another adhesive film.

In Figure 1 the waterproofing material 2 is passed between pressing rolls 4, which form it into sheet or strip form. This strip of formed material then passes between an upper fiber applying device 6, which drops the fibers upon the upper surface of the asphaltic sheet of material, and a lower fiber applying wheel 8, which rotates adjacent and into a container of fibers and picks them up and applies them to the under surface of the traveling sheet, the waterproofing material with the fibers applied to its upper and lower surface then traveling between the pressing rolls 10, which presses the fibers into the adhesive surface of the sheet or strip of traveling material.

In Figure 2 of the drawing the waterproofing material is fed between the rolls 12 and formed into sheets, thence passing between the coating rolls 14, which coat the same with a suitable adhesive, such for instance as a suitable varnish that dries to a flexible waterproof film. The strip of material then passes between air blowing devices which blow the fibers upon the upper and lower surfaces of the traveling strip, and thence it passes thru the pressing rolls 18, which press the fibers into the strip and into the adhesive film, and finally the strip thus formed passes between the coating rolls 20, which apply an additional or superficial coating of this drying adhesive, heretofore described in the specification.

It will, of course, be evident that instead of using a set of pressing rolls for forming the waterproofing material into strip form I may use any other type of means, such for instance as an extruding machine 22, shown in Figure 3 of the drawings.

In Figure 4 of the drawings the waterproofing material 2 is shown with the fibers 24 applied to the sides thereof.

In Figure 5 the waterproofing material 2 is shown as coated with an adhesive film 26, and the fibers 24 are adhered to this film.

In Figure 6 the second adhesive film 28 is shown as lying over the fibers 24, which are adhered to the inner adhesive film 26.

I do not wish to be limited to the nature of the binder, just so the binder is waterproofed and preferably one that is more or less elastic and does not become brittle.

While I prefer asbestos fiber of length, asbestos fiber may be made to answer the purpose, or animal hair.

In some constructions it is also desirable to coat over the fibers after being impressed into the adhesive layer in order to properly water-

proof them. In this manner the strength of the fibers is not interfered with because they are not penetrated and they have their own tensile strength, whereas if they are previously treated with a degumming treatment mixed with a saturant the fiber will lose much of its binding strength.

Another disadvantage in preparing a saturated reinforcing felt side is that the fibers are disintegrated and comminuted. Furthermore, they are mostly cotton fibers and are readily saturated with the saturant. On the contrary, by my method I secure the advantage of the original strength of the fibers and prevent saturation, thus obtaining the full effect of their reinforcing value. A further advantage resides in the fact that I am able to use binders which are not suitable for roofing felt purposes or saturated felt, and in fact which would be too expensive, and therefore obtain a much stronger reinforcing sheet. I likewise economize in preparing my reinforcement because I do not first have to manufacture and prepare reinforcing sheets and later apply them to the joint. My reinforcing medium is made up in processes and can therefore be effected more economically, and a much wider range of fibers can be employed, as well as a much wider range of binders.

I claim:

1. As an article of manufacture a pre-formed strip composed of a waterproof binder of substantial thickness, said body having upon its outer faces an adhesive film having linear fibers imbedded therein.
2. As an article of manufacture a pre-formed strip composed of a waterproof binder of substantial thickness, said body having upon its outer faces an adhesive film having linear fibers pressed therein, and an adhesive coating film applied over the linear fibers.
3. An expansion joint, the main body of which is of substantial thickness comprising homogeneous mixture of waterproof binder and fiber, having upon its outer face a film of waterproof adhesive having attached thereto linear fibers.
4. An expansion joint, the main body of which is of substantial thickness comprising a homogeneous mixture of waterproof binder and fiber, having upon its outer face a film of waterproof adhesive having linear fibers imbedded therein, and an adhesive coating film applied over the linear fibers.
5. A prepared expansion strip comprising a waterproof binder and a filler, said strip having a film of waterproof adhesive on its outer surface and fibers of linear dimension imbedded therein, and an adhesive coating film applied over the linear fibers.
6. A prepared expansion strip comprising a waterproof binder and a filler, said strip having a film of waterproof adhesive on its

outer surface and fibers of linear dimension extraneously pressed therein.

7. The method of preparing a preformed expansion strip in which a waterproof binder is pressed into sheet form and before the surface has become set applying thereto fibers of linear dimension, and pressing said fibers into the surface of the strip.

8. The method of preparing a preformed expansion joint by preparing a body strip in sheet form, applying to the outer faces of said sheet before it has time to set a waterproof adhesive film, and applying to said film fibers of linear dimension.

9. The method of preparing preformed expansion joint by preparing a body strip in sheet form, applying to the outer faces of said sheet before it has time to set a waterproof adhesive film, and applying thereto fibers of linear dimension and pressing said fibers into the surface of the film.

10. The method of preparing a preformed expansion joint by preparing a body strip in sheet form, applying to the outer faces of said sheet before it has time to set a waterproof adhesive film, and applying thereto fibers of linear dimension, said film setting and tenaciously holding the fiber in its surface.

11. The method of preparing an expansion joint by preparing a main body in sheet form, applying to the face of said sheet a waterproof adhesive binder, imbedding linear fibers in said adhesive binder, pressing the fibers therein, then coating over said fibers with another adhesive binder imbedding said fibers in the binder.

12. The method of making preformed constructional material characterized by forming a waterproof body strip, applying fibers to the surface of the strip before same becomes set, and pressing the fibers into the surface of said strip.

Signed at Chicago, Illinois, this 12th day of August, 1927.

ALBERT C. FISCHER.

115

120

125

130